

April 20, 1948.

C. G. SILVERBERG

2,440,187

REFRACTORY AND METHOD OF MAKING THE SAME

Filed Jan. 16, 1943



Fig. 1

Fig. 2



Fig. 3

Fig. 4



Fig. 6

INVENTOR  
CARL G. SILVERBERG  
BY  
Louis B. Gagnon  
ATTORNEY

## UNITED STATES PATENT OFFICE

2,440,187

REFRACTORY AND METHOD OF MAKING  
THE SAMECarl G. Silverberg, Brookfield, Mass., assignor to  
American Optical Company, Southbridge,  
Mass., a voluntary association of Massachusetts

Application January 16, 1943, Serial No. 472,604

13 Claims. (Cl. 106—66)

**1**  
This invention relates to refractory devices and has particular reference to novel means and methods of making the same.

One of the principal objects of the invention is to provide a refractory device for supporting an article to be heated whereby the said device inherently possesses characteristics which will obviate any tendency for the article being heated to adhere to the refractory device during said heating operation and has particular reference to novel means and methods of making the same.

Another object is to provide refractory devices of the above character which are particularly adaptable for use in supporting a glass article during heating whereby the resultant article will more accurately respond to the heat treatment and will be of more uniform shape resulting from said heat treatment.

Another object is to provide refractory devices of the above character which may be more accurately controlled as to surface shape whereby a glass blank supported by said article and subjected to heat treatment with a view to dropping said blank to the surface shape of said device may be more efficiently and uniformly formed with less tendency of the glass material of said blank adhering with the refractory device during said heat treatment.

Another object is to more uniformly control the distribution of heat during the heating operation.

Another object is to provide refractory devices of the above character inherently possessing means for more positively controlling the distribution of heat during the use of the device and which will enable the heating operations to be performed with a requirement of a minimum of time as compared with prior art methods.

Another object is to provide refractory devices of the above character enabling the heating operations to be performed in a minimum of time and with less tendency of breakage of the article or the block during said heating operation.

Another object is to provide novel means and methods of forming refractories of the above character whereby the supporting surface shape of the refractory may be more positively and accurately controlled.

Another object is to provide refractory devices of the above character whereby the supporting surface shape may be altered after the main refractory device has been fabricated.

Other objects and advantages of the invention will become apparent from the following description taken in connection with the ac-

**2**  
companying drawings and it will be apparent that many changes may be made in the details of construction, arrangement of parts and steps of the methods shown and described without departing from the spirit of the invention as expressed in the accompanying claims. I, therefore, do not wish to be limited to the exact details of construction, arrangement of parts and methods shown and described as the preferred forms only have been given by way of illustration.

Referring to the drawings:

Fig. 1 is a sectional view through a mold block illustrating one step in the process of manufacture;

Fig. 2 is a view generally similar to Fig. 1 illustrating a further step in the process of manufacture;

Fig. 3 is a longitudinal sectional view of a modified form of molding device;

Fig. 4 is a sectional view taken as on line 4—4 of Fig. 3 and looking in the direction indicated by the arrows;

Fig. 5 is a sectional view generally similar to Figs. 1 and 2 with a further modification of the invention; and

Fig. 6 is a diagrammatic illustration of a refractory block in use in supporting an article to be dropped in the furnace.

It has been usual in the past to form refractory blocks or refractory devices of the character described of silicon carbide which, at low heating temperatures, produces fairly satisfactory results but in many instances, particularly when joining two or more pieces of glass together by fusion and at the temperature required for said fusion, difficulty was encountered in having the glass engaging the refractory adhering to the surface of the refractory. In order to overcome or reduce the above difficulty, it has been necessary in most instances in the past to treat the surface of the refractory, as by dusting with clay or graphite. This requirement rendered such prior art refractories impractical for use in dropping glass blanks or articles to controlled surface curvatures as, in most instances, the particles of the dusting material present on the supporting surface of the refractory caused surface distortions in the dropped article. This also introduced difficulty in fusion as one of the essentials to successful fusing is that the atmosphere be as free from dust particles as possible during the assembling of the parts to be fused and during the actual fusing operation. It is quite apparent, when such dusting of the supporting surface is required, that

40  
45  
50  
55

the particles of the dusting material might be deposited on the surfaces of the glasses to be fused with the danger of ruining the fusing operation.

The above difficulties have been definitely overcome by the present invention in that the refractory devices embodying the invention do not require dusting as they inherently possess characteristics which will permit the use of high temperatures with no danger of adhesion of the surface of the glass article in engagement with the refractory device.

Another advantage of the present invention is that the distribution of the heat may be controlled during the heating operation.

A still further advantage is that the surface shapes of the dropped or heated articles may be more positively controlled during said heating so that the resultant surface of the article will be more optically accurate than has hitherto been possible to obtain.

Another advantage is that the initial fabrication of the refractory may be more efficiently performed.

Referring to the drawings wherein like characters of reference designate like parts throughout the several views, the major ingredient used in forming the refractory is kyanite. This ingredient has initially dry characteristics but by proper milling and reducing of said ingredient to fine powdered form and by the addition of a small amount of water, it is possible to shape the material to the shapes desired. It has, however, been found that the addition of plastic clay of any of the various refractory ball clays which will not introduce vitrification may be added as a binder to greatly facilitate the fabrication of the refractory. It is to be understood that any mention of ball clay hereinafter refers to a refractory clay having plastic characteristics.

The addition of sodium silicate to the above ingredients introduces greater ease of fabrication. As a further aid, sodium carbonate may be added. Sodium silicate and sodium carbonate are added mainly to introduce greater dispersive characteristics and to facilitate ease in handling the resultant compound.

To further stabilize the compound a small amount of triethanolamine may be added. This, of course, depends upon the method of fabrication of the article and will provide additional dispersive characteristics. To reduce the compound to a more fluid state water may be added. The amount of water to be used will be determined by the method of fabrication employed.

One of the preferred compositions is as follows:

|                       | Grams | Approximate Parts by Weight |
|-----------------------|-------|-----------------------------|
| Kyanite.....          | 3,200 | 8,000                       |
| Ball Clay.....        | 800   | 2,000                       |
| Sodium Carbonate..... | 4     | 10                          |
| Sodium Silicate.....  | 2     | 20                          |
| Triethanolamine.....  |       | 5                           |
| Water.....            | 1,000 | 2,500                       |

The above produces a fluid composition which is particularly suitable for pouring in molds, such as illustrated in Figs. 1 through 4.

Although the preferred composition has been found to be substantially that set forth above, it is to be understood that the amount of ball clay may be varied from 0 to 35% of the total composition.

Kyanite has a tendency to expand on heating 75 water.

while ball clay has a tendency to shrink so that by controlling the proportions of each according to their tendencies to shrink or expand one can be made to overcome the other so that a more definite size control can be maintained.

The amount of sodium silicate and sodium carbonate must be maintained at a minimum to prevent fluxing and possible adhesive characteristics in the resultant refractory. The amount of said materials used therefore is only that which is sufficient to bring about the desirable working characteristics and said characteristics can be accomplished without the introduction of any adhesive characteristics. Although sodium silicate, sodium carbonate and triethanolamine have been set forth above as good dispersing agents, it is to be understood that any one or all of said materials may be replaced by one or more of the following ingredients:

20 Morpholine, lignin, sodium gallate, etc. Tannic acid or any other known dispersive agent or agents.

With proper temperature and time controls, a refractory formed of the above materials or compositions will produce very satisfactory results with no danger of adhesion of glass or material of the article being dropped with the refractory during the heating operation.

25 It has been found, however, that much more satisfactory results can be obtained by the addition of chrome oxide, rouge, manganese dioxide or other known ceramic colorants which do not produce vitrification to any one of the refractory compositions set forth above. The preferred ingredient, however, is chrome oxide which, in a preferred composition, comprises 0 to 25% replacing kyanite in the body, that is, when chrome oxide or one of the other colorants set forth above are used, the kyanite is reduced correspondingly. The purpose of adding the above colorants to the refractory composition is to more uniformly control the distribution of heat throughout the article being supported and also throughout the refractory itself. The above colorants are infra-red absorbing materials which during the heating of the article being supported tends to absorb the heat. This absorption of the radiant heat provides a more uniform heating of the refractory.

30 It is to be noted that green chrome oxide is set forth above as the preferred infra-red absorbing ingredient. It is to be understood, however, that rouge or manganese dioxide may be used. It has been found that when rouge or manganese dioxide is used the initial refractory produces very satisfactory results but upon repetitive use the said refractories tend to lose their efficiency as to infra-red absorption. In instances, however, when the said refractories are not required for repetitive use such infra-red absorbing ingredients are practical for use but in instances when the refractories are for repetitive use green chrome oxide produces much more satisfactory results.

35 In addition to introducing the desired infra-red absorbing characteristics, such ingredients introduce a greater resistance to adhesion in the resultant device. This is particularly true of green chrome oxide.

40 One of the preferred methods of forming the composition is as follows:

A. First dissolve one or more of the dispersing agents set forth above in the required amount of

B. Add ball clay of the amount required depending upon the amount of kyanite to be used. If the said clay is in lump form it is allowed to soak until the lumps may readily be broken up. The resultant mixture is thoroughly stirred.

C. The required amount of colorant or infrared absorbing material is then placed in the mixture and thoroughly stirred therein. The preferred colorant being green chrome oxide.

D. The kyanite is then added while mixing as fast as the mixture will disperse the said kyanite without forming large lumps. The resultant mixture will be fairly smooth.

E. To the above, although not absolutely essential, a small amount of triethanolamine is added to the batch or mix.

The mixture resulting from the combining of the above ingredients is then preferably milled in a suitable ball mill or the like for a period of about 70 to 80 hours. The mixture is then ready for use.

The preferred composition is substantially as follows:

|                      |       |      |
|----------------------|-------|------|
| Kyanite              | grams | 2400 |
| Ball clay            | do    | 800  |
| Chrome oxide (green) | do    | 800  |
| Sodium carbonate     | do    | 4    |
| Sodium silicate      | do    | 8    |
| Triethanolamine      | cc.   | 2    |
| Water                | grams | 1000 |

If the said mixture is to be kept for some time prior to its being used a small amount of formaldehyde solution is added, either before or after the milling, as a preservative. Approximately 1 cc. of 40% formaldehyde solution, added to the preferred batch set forth above has been found to produce desirable results. It is to be understood that the said mixture is preferably placed in a closed container to prevent evaporation and loss of moisture.

In Fig. 1 there is illustrated a mold member 6 suitable for use with a fluid mixture such as set forth above. This mold member is preferably formed of plaster of Paris or other suitable porous material and is provided with a recess 7 having its internal walls and bottom 8 formed substantially to the shape desired of the resultant refractory. A suitable amount of fluid composition 9 is poured into the recess and due to the porosity of the plaster of Paris or other similar material from which the mold 6 is formed a certain amount of the water is absorbed by the said porous material, particularly, throughout the surfaces which are in contiguous relation with the fluid composition 9. This action causes a superficial hardening of the composition throughout said surfaces tending to build up to a considerable thickness when allowed to set for a relatively short period of time. It has been found that if the mold is relatively dry and porous that within a period of 15 minutes a wall thickness suitable for small articles will be built up. The fluid which has not reached a solid state is then poured from within the built-up wall of the composition leaving a central cavity 10, as shown in Fig. 2. The material which has been removed from the cavity may be used for other refractories. If desired, however, the entire deposit 9 may be allowed to harden in the mold. Further hardening or drying out of the composition will cause the material of said composition to contract whereby the resultant refractory may be easily removed from the mold. The contraction will take place throughout all of the contiguous surfaces.

The above is a very simple form of mold and is used in instances when only one shape of surface is desired.

In instances when the opposed sides of the supporting block are to be shaped to a given shape a mold similar to that shown in Figs. 3 and 4 may be used, this mold comprising a plurality of spaced blocks 11 held in spaced relation with each other by a band of metal or other suitable material 12 which is inserted within a suitable retaining block 13. The band 12 is provided with spaced deflected lip portions 14 which provide means for gaining access to the interior of the mold between the blocks 11. The blocks 11 may be formed of plaster of Paris or other porous materials such as set forth above. The blocks 11 are placed in spaced relation with each other by the amount required of the resultant thickness of the refractories and by providing a plurality of spaced blocks several refractories may be formed in a single casting operation. The fluid composition is poured inwardly of the mouth formed by the spaced lips 14 between the blocks 11. The composition is allowed to remain in the mold until it has reached a desirable hardened state whereby the contiguous surfaces of the blocks and the composition are separated through the contraction of the composition. The blocks together with the molded refractories are then slid outwardly of the retaining block 13. The band 12 is then removed whereby the several blocks and resulting refractories may be separated. After each casting operation the blocks 11 have to be dried out so as to have the proper porosity.

In Fig. 5 there is diagrammatically illustrated another method of forming the refractories. In this view, there is illustrated a die member 15 in which the composition 16 to be molded is placed and a suitable plunger 17 is provided for compressing the material inwardly of the cavity of the die. In this instance, the composition does not have the fluidity of the above mentioned composition. Less water is used and the composition is in the form of a distortable mass 16. The amount of the composition 16 is controlled according to the resultant size of the refractory desired. It is to be understood that the die 15 is provided with an inner surface 18 which is substantially the shape desired of the supporting surface of the refractory. Upon removal of the shaped refractory members from the dies or molds, set forth above, the said refractories are preferably initially placed within a furnace, such as an electrical furnace or the like, at a temperature sufficient to slowly remove all of the free water which might be present in said initially shaped refractories. This drying operation may be accomplished at room temperature but may be hastened by the above procedure, it being understood, of course, that care must be taken that the temperature is not too high so as to cause the disintegration of the refractories through the formation of steam during said drying and care must also be taken that the drying takes place substantially uniformly throughout the refractories. The dried refractory blocks, if placed in water, will have a tendency to disintegrate and, therefore, must be fired at a higher temperature. This firing is accomplished by increasing the temperature of the heat in the furnaces in which the drying operation has been performed or by placing the said dried refractories in another furnace or suitable heating de-

vice. The firing schedule for a small furnace is about as follows:

From room temperature to 400° F. by raising the temperature at 100° F. per hour  
200° F. per hour to 800° F.  
400° F. per hour to 2200° F.

The furnace is held at 2200° F. for approximately five hours. If smaller furnace is used temperature rates would be increased and time decreased, if larger articles are made the temperature changes must be very much slower and time intervals lengthened.

From the above, it will be seen that the temperatures are increased gradually until the desired maximum temperature is obtained. This firing is for the purpose of bringing about a positive bond between the particles of the composition tending to produce a refractory having the desired supporting characteristics.

Although the temperature schedule set forth above gives the 2200° F. temperature as the high limit it is to be understood that higher or lower temperatures may be used for the final temperature. The upper temperature limit, however, must be such as to avoid vitrification or the formation of any glassy phase in the refractory. The firing temperature, however, which will produce vitrification is much above that required in the subsequent heating of articles which are to be supported and dropped through the action of heat so that there will be no inherent danger of vitrification taking place during the actual use of the refractory. Firing at relatively low temperatures, say below 1800° F., causes the resultant refractory to be relatively soft and less resistant to wear and breakage. Above 1800° F. and at approximately 2200° F. the refractory is much more resistant to wear and to breakage and yet is of such a nature that the supporting surface may be readily shaped by grinding or other suitable means. When the firing temperature is increased considerably above 2200° F. there is not only a danger of vitrification of the composition but there is a danger of deformation during firing and the introduction of extreme brittleness and difficulty in shaping. However, for certain purposes we have found that temperatures above 2200° F. may be desirable, especially when increased hardness is desired. One particularly desirable temperature is 2250° F.

The composition set forth above is of such a nature that even after firing the supporting surface or surfaces of the refractory may be built-up through the use of an additional amount of unfired composition. This is particularly important when portions of the supporting surface are required to be altered to obtain more accurate shaping. This is accomplished by first saturating the refractory block with water or more particularly the surface thereof which is to be built-up. A given amount of unfired composition is then placed on the supporting surface in the vicinity which is to be built-up. The said built-up portion is then shaped to the resultant shape desired and the block is then initially dried and subsequently fired in the above manner. If there is to be an appreciable amount of building up this may be accomplished through successive stages in the above manner. This is found particularly useful when the refractory has been accidentally scratched or otherwise injured.

In Fig. 6 there is diagrammatically illustrated a furnace 19 having suitable heating coils 20 therein. Internally of the furnace 19 there is

shown a refractory block 21 formed by any of the methods set forth above. This refractory block has a supporting surface 22 thereon formed either during the fabrication of the block or by subsequent shaping. On the supporting surface 22 there is shown an article 23 to be dropped by heating. The article 23 may be a glass blank which is to be heated to a temperature sufficient to cause the material of said blank to drop through gravitational action and conform to the surface shape of the supporting surface 22. It is to be understood that instead of using the refractory 21 for the purpose of dropping a blank, such as set forth above, the said refractories may be used for several other operations, for example, for supporting a major blank during the fusion of a minor blank thereto as is common practice in the forming of bifocal or multifocal ophthalmic lenses. The refractory block is of such a nature that the surface of the article engaging the supporting surface of the refractory 22 will have no tendency to adhere to said supporting surface and does not require the use of additional materials as a preventative for said adherence.

Another very desirable characteristic of the present invention is that the refractories do not become altered or distorted as to shape through continued use.

Although kyanite is set forth as the preferred major constituent it is to be understood that andalusite or sillimanite may be substituted for such kyanite or mixtures of andalusite, kyanite, and sillimanite may be used. Clays or other ingredients having an alumina content approaching kyanite may also be used. Care should be taken, however, that the temperatures used in firing and that the temperatures at which the said resultant refractories are to be used are below that which would cause vitrification.

In instances where high alumina content ingredients are used, such as high alumina clays it might be necessary to subject the said ingredient to an initial firing or dehydration process. This, however, is not essential with the kyanite, andalusite and sillimanite materials as these materials are inherently anhydrous.

Kyanite, andalusite and sillimanite have characteristics which are such that no vitrification takes place within the range of temperatures to which they are to be used in the present instance as the articles which are to be heat treated are in most instances glass articles.

The above mentioned ingredients, kyanite, andalusite, and sillimanite are aluminum silicates which inherently contain no water of crystallization and are given herein as examples of ingredients which are suitable for forming refractories of the character described. They are all anhydrous aluminium silicate minerals having an alumina silica ratio of approximately 1 to 1, that is, 1  $\text{Al}_2\text{O}_3$  and 1  $\text{SiO}_2$ .

From the foregoing description it will be seen that simple, efficient and economical means and methods have been provided for accomplishing all of the objects and advantages of the invention.

Having described my invention, I claim:

1. The method of forming a refractory suitable for heat dropping glass articles comprising forming a mixture of an ingredient having a high aluminous silicate content in substantially anhydrous state, ball clay, an infra-red absorbing ingredient and water with the ingredient of high aluminous silicate content being in excess of the ball clay and the infra-red absorbing ingredient being controlled according to the infra-

red absorbing characteristics desired, shaping said composition to produce a refractory having a supporting surface of substantially the shape desired to be formed on the glass article, subjecting said shaped refractory to heat of a relatively low temperature to remove the water and subsequently subjecting said refractory to heat of a relatively high temperature with the maximum temperature being substantially above the temperature at which the glass articles will initially soften and controlled to introduce the proper binding action of the ingredients of the composition with no vitrification and so that a non-vitrified body substantially non-adhesive to glass in the presence of heat sufficient to soften the glass remains.

2. The method of forming a refractory suitable for heat dropping glass articles comprising forming a mixture of an ingredient having a high aluminous silicate content in substantially anhydrous state, ball clay, green chrome oxide and water with the ingredient of high aluminous silicate content being in excess of the ball clay and the green chromic oxide being of an amount to introduce the infra-red absorbing characteristics desired, shaping said composition to produce a refractory having a supporting surface of substantially the shape desired to be formed on the glass article, subjecting said shaped refractory to heat of a relatively low temperature to remove the water and subsequently subjecting said refractory to heat of a relatively high temperature being substantially above the temperature at which the glass softens and with the maximum temperature controlled to introduce the proper binding action of the ingredients of the composition with no vitrification and so that a non-vitrified body substantially non-adhesive to glass in the presence of heat sufficient to soften the glass remains.

3. A refractory having a surface of controlled shape for supporting a glass article to be dropped thereon under the action of heat that is substantially non-adhesive to said article in the presence of heat of an amount sufficient to soften the article, said refractory comprising a non-vitrified body consisting of a mixture of kyanite and ball clay with said kyanite being in excess of said ball clay and with the said mixture containing a dispersing agent and an ingredient having infra-red absorbing characteristics, the ingredients of said mixture being heat joined with each other at a temperature above the softening point of the article to be softened but below the point of vitrification of said mixture.

4. A refractory suitable for use in dropping glass articles comprising a non-vitrified body substantially non-adhesive to said article in the presence of heat of an amount sufficient to soften said article, said body being formed hollow and with a top portion of substantially uniform thickness having a supporting surface of a shape controlled to impart the shape desired to a surface portion of said article, said body consisting of kyanite, ball clay and green chrome oxide as an added infra-red absorbing ingredient with the kyanite being in excess of said ball clay and green chrome oxide and with the amount of said green chrome oxide being controlled according to the infra-red absorbing characteristics desired.

5. A refractory for use in supporting glass at softening temperatures and non-adhesive to said glass at said temperatures, comprising essentially a highly refractory aluminous silicate ma-

terial combined with green chrome oxide of an amount sufficient to produce long wave infra-red absorption and containing suitable non-vitrifying bonding material with said ingredients being bonded with each other at a temperature substantially above the temperature at which the glass to be supported will soften but substantially below the temperature at which any fusion or vitrification of the ingredients takes place.

6. A refractory for use in heat dropping glass articles that is non-adhesive to the articles in the presence of heat sufficient to soften the articles, said refractory comprising a plurality of heat joined ingredients including as a major ingredient a high alumina mineral, ball clay as a binder of an amount which, with the temperature required to produce said heat joining, will introduce greater ease of fabrication with no vitrification, a dispersing agent and a colorant of an amount for introducing desired infra-red absorbing characteristics, the heat joining temperature being substantially above the temperature required for said heat dropping of said glass articles but being below the temperature at which fusion or vitrification of the ingredients takes place.

7. A refractory for use in heat dropping glass articles that is non-adhesive to the glass at the softening temperature thereof consisting essentially of a highly refractory aluminous silicate mineral combined with green chrome oxide upwardly to approximately 25% depending upon the infra-red absorbing characteristics desired, said ingredients being heat joined with each other at a temperature such that no vitrification takes place but substantially above the temperature at which the articles with which the refractory is to be used softens.

8. A refractory suitable for use in heat dropping a glass article that is substantially non-adhesive to the glass in the presence of heat sufficient to soften the glass, said refractory comprising a body portion essentially of kyanite in combination with ball clay of from 0 to 35% of the total composition and green chrome oxide of an amount upwardly to approximately 25% depending upon the infra-red absorbing characteristics desired, and containing as a deflocculent sodium silicate and sodium carbonate, said ingredients being heat joined with each other at a temperature substantially above the softening point of the glass article with the amount of sodium silicate, sodium carbonate and the temperature of heating being so controlled as to avoid fluxing and so that the resultant refractory is free from a glassy phase and possesses non-adhesive characteristics as to the glass article being dropped in the range of temperatures at which the glass softens sufficiently to drop.

9. The method of forming a refractory suitable for heat dropping glass articles comprising forming a mixture of kyanite, ball clay, green chrome oxide and water with the green chrome oxide being controlled according to the infra-red absorbing characteristics desired, shaping the composition to the shape of the refractory desired, subjecting said refractory to heat of a relatively low temperature to remove the water and subsequently subjecting the said refractory to heat of a temperature substantially above the temperature at which the glass articles soften and controlled so as to introduce a proper binding of the ingredients with no vitrification.

10. A refractory suitable for use in heat drop-

## 11

ping glass articles comprising a body portion embodying

|                    |       |      |
|--------------------|-------|------|
| Kyanite            | grams | 2400 |
| Ball clay          | do    | 800  |
| Green chrome oxide | do    | 800  |
| Sodium silicate    | do    | 8    |
| Sodium carbonate   | do    | 4    |
| Triethanolamine    | cc    | 2    |
| Water              | grams | 1000 |

11. A refractory for use in heat dropping glass blanks that will be substantially non-adherent to the glass of the blanks in the presence of heat sufficient to soften said glass comprising a body portion embodying substantially:

Per cent by weight

|                    |    |
|--------------------|----|
| Kyanite            | 60 |
| Ball clay          | 20 |
| Green chrome oxide | 20 |

12. A refractory for use in heat dropping glass blanks that will be substantially non-adherent to the glass of the blanks in the presence of heat sufficient to soften said glass comprising a body portion embodying substantially:

Per cent by weight

|                                        |    |
|----------------------------------------|----|
| A highly refractory aluminous material | 60 |
| Ball clay                              | 20 |
| Green chrome oxide                     | 20 |

13. A refractory for use in heat dropping glass articles that is substantially non-adhesive to the articles in the presence of heat sufficient to soften the articles, said refractory comprising a plurality of heat joined ingredients including as a major ingredient a high alumina mineral, ball clay as a binder of an amount which, with the temperature required to produce said heat joining, will introduce a greater ease of fabrication with no vitrification, and a colorant of an amount for introducing desired infra red absorbing characteristics, the heat joining tempera-

## 12

ture being substantially above the temperature required for said heat dropping of said glass articles but being below the temperature at which vitrification of the ingredients takes place.

CARL G. SILVERBERG.

## REFERENCES CITED

The following references are of record in the file of this patent:

## UNITED STATES PATENTS

| Number       | Name           | Date           |
|--------------|----------------|----------------|
| 94,726       | Eaton          | Sept. 14, 1869 |
| 15 637,635   | Mersch         | Nov. 21, 1899  |
| 700,673      | Buchner        | May 20, 1902   |
| 1,081,536    | Jeppson        | Dec. 16, 1913  |
| 1,292,953    | Jeppson et al. | Jan. 28, 1919  |
| 1,631,695    | Riddle         | June 7, 1927   |
| 16 1,682,675 | Horsfield      | Aug. 28, 1928  |
| 1,712,005    | Lambie et al.  | May 7, 1929    |
| 1,716,395    | Trostel        | June 11, 1929  |
| 1,760,360    | Hood           | May 27, 1930   |
| 1,769,297    | Lambie et al.  | July 1, 1930   |
| 20 1,812,376 | Ross et al.    | June 30, 1931  |
| 1,856,613    | Ackermann      | May 3, 1932    |
| 1,897,183    | White          | Feb. 14, 1933  |
| 1,909,785    | McDougal       | May 16, 1933   |
| 1,942,879    | Riddle         | Jan. 9, 1934   |
| 30 2,079,715 | Pole           | May 11, 1937   |
| 2,159,349    | Bennett        | May 23, 1939   |
| 2,160,873    | Kerla          | June 6, 1939   |
| 2,207,558    | Singer         | July 9, 1940   |
| 2,270,607    | Ryschkewitsch  | Jan. 20, 1942  |
| 35 2,272,039 | Morgan         | Feb. 3, 1942   |
| 2,308,473    | Wadman et al.  | Jan. 12, 1943  |
| 2,331,232    | Ross           | Oct. 5, 1943   |

## FOREIGN PATENTS

| 40 Number | Country | Date |
|-----------|---------|------|
| 676,595   | Germany | 1939 |